

Oct. 2, 1928.

1,686,150

C. G. FINK ET AL

ABRASIVE SURFACE AND METHOD OF MAKING SAME

Filed March 14, 1927

*Fig. 1,*



*Fig. 2,*



*Fig. 3,*



*Colin G. Fink  
Arthur H. Rapp  
INVENTORS*

*Roger Kennedy, Campbell  
ATTORNEYS*

Patented Oct. 2, 1928.

1,686,150

# UNITED STATES PATENT OFFICE.

COLIN G. FINK AND ARTHUR H. KOPP, OF NEW YORK, N. Y., ASSIGNEES TO AMERICAN ABRASIVE METALS COMPANY, A CORPORATION OF NEW YORK.

## ABRASIVE SURFACE AND METHOD OF MAKING SAME.

Application filed March 14, 1927. Serial No. 175,353.

The invention relates generally to articles adapted to resist abrasion and more particularly to articles having a body of metal and a resistant surface formed by embedding therein hard mineral or wear-resisting elements, such as corundum, emery, and the like.

A well known method of making articles adapted to resist abrasion, such for example, 10 as stair treads, conduits for dredging pumps, ash conveyors, and the like, consists in forming a mold, placing a layer of wear-resisting elements, such as grains of carborundum, corundum, alundum, emery, or the like, upon 15 a surface of the mold adapted to shape a surface of the article to be made, and pouring molten metal into the mold. The resulting product is an article of the shape or form desired to suit the particular purpose, 20 as a stair tread, with a body of metal and a tread surface in which are embedded the grains of the wear-resisting material, as emery. It is important that these grains of the wear-resisting material should be firmly 25 and closely gripped by the surrounding metal in which they are embedded, because if any of the grains should be separated from their metal base, due to the rough usage to which the article is subjected, the surface thus 30 bared of the protecting grains would be speedily worn away, and thus other adjacent grains would also be rendered liable to be separated from their metal bed.

The present invention, therefore, has for 35 an object to provide an article of the character described which will be proof against the loss of the wear-resisting grains, and the invention also includes within its purview the method of producing such articles.

40 In the accompanying drawings, which are referred to herein and form part hereof,

Fig. 1 is a cross-section of a mold adapted to produce a stair-tread having the characteristics of the invention;

45 Fig. 2 is a perspective view of a stair-tread produced in such mold in accordance with the method of the invention; and

50 Fig. 3 shows some of the grains of the wear-resisting material, prepared according to the invention, to be placed in said mold and incorporated in the surface of the article.

An article of the character described having a wear-resistant surface may have a body 55 portion composed of any suitable material

adapted to meet the requirements of the particular use to which the article is to be put. In a stair-tread, for example, the body may be of a metal, as iron, which has the required strength and rigidity for its purpose and which can be cast into the desired form. As has been stated, however, in order to make for the highest efficiency, the material in which the grains of wear-resisting material are embedded should be of such a nature as to cling closely to the grains and grip them in a firm and enduring embrace. Because of their peculiar characteristics, however, the grains of wear-resisting material mentioned do not lend themselves readily to the described close embrace by certain materials otherwise eminently suitable to form the body of the article in which the grains are to be embedded, as, for instance, iron in the casting process described. 70 The invention, therefore, contemplates providing a means and method for bringing about this desired affinity between the grains of wear-resisting material and the material forming the body of the article, as the cast 75 iron. This is accomplished by interposing between each grain and the body of the article a material which will adhere closely to the grain and at the same time combine with the body of the article, said material being 80 of such nature that, when so interposed and combined, a secure anchorage for the grain will be provided. Hence, according to the preferred way of carrying out the invention, the grains of wear-resisting material before 85 being placed in the mold are coated with a metal which has a lower melting point than, and which will form at such lower temperature a localized hard alloy with, the iron, for example, forming the body of the article. 90 A suitable metal for this purpose is tin and although tin is soft, it has been found that a thin coating of tin on the grains will form a localized hard alloy with the iron of the body of the article and so secure the grains 95 from disturbance. A simple way of providing the grains with this thin coating is to use friction, and therefore the grains with surfaces preferably roughened by fused alkali are placed in a drum with a supply of 100 small pieces of tin and tumbled until they are properly coated. The grains are now 105 ready to be placed in the mold.

Referring now to the drawings in detail, there is shown in Fig. 1 a mold 4, compris- 110

ing a drag 5 and cope 6 which are formed to mold a stair-tread 7 which will be here described, together with the method of making the same, to illustrate the invention.

6 On a surface 8 of the mold 4, which surface is adapted to shape the resistant surface of the tread 7, is placed a layer of grains 10 of emery. These grains 10, as shown in Fig. 3, have previously been provided by 10 the tumbling process with a thin coating of tin. Thru the gate 11 of the mold the molten iron is poured and flows over and about the grains 10 and thus form the body 12 of the tread with its resistant surface 15 13, as shown in Fig. 2. As the molten iron surrounds the grains, the iron will form with said coating a localized thin, hard alloy which will "wet" or cling closely to the surfaces of the grains, which will now be 20 securely embedded in the surface of the tread. Other articles adapted to resist abrasion may be made in a similar way.

The invention in its broader aspects is not limited to the particular metals or alloy 25 referred to nor to the particular order or sequence of steps by which the method of making the article is carried out, as different metals may be used and the order of the successive steps of the method changed without departing from the main principles of the invention or sacrificing its chief advantages.

We claim:

1. An article adapted to resist abrasion 35 comprising a base of cast metal, grains of wear-resisting material embedded in the surface of said base, and a localized metal alloy immediately surrounding each of said grains, the remainder of said base being free 40 of said alloy.

2. An article adapted to resist abrasion comprising a base of cast metal, grains of wear-resisting material embedded in the surface of said base, and a localized thin 45 metal alloy immediately surrounding each of said grains, the remainder of said base being free of said alloy.

3. An article adapted to resist abrasion comprising a base of cast metal, grains of wear-resisting material embedded in the surface of said base, and a localized metal alloy immediately surrounding each of said grains, the said alloy being composed of the metal of the body of the base and a metal 55 having a lower melting point than the said body metal, the remainder of said base being free of said alloy.

4. An article adapted to resist abrasion comprising a base of cast metal, grains of wear-resisting material embedded in the surface of said base, and a localized alloy of 60 tin and iron immediately surrounding each of said grains, the remainder of said base being free of said alloy.

5. An article adapted to resist abrasion

comprising a base of cast iron, grains of wear-resisting material embedded in the surface of said base, and a localized alloy of tin with the iron of the base immediately surrounding each of said grains, the remainder 70 of said base being free of said alloy.

6. An article adapted to resist abrasion comprising a base of cast iron, grains of wear-resisting material embedded in the surface of said base, and a localized thin 75 alloy of tin with the iron of the base immediately surrounding each of said grains, the remainder of said base being free of said alloy.

7. The method of producing an article 80 adapted to resist abrasion, which method includes forming a mold for the article, applying a coating of metal to grains of wear resisting material, distributing a layer of said previously coated grains on a surface 85 of said mold adapted to shape a surface of said article, and pouring molten metal into said mold.

8. The method of producing an article 90 adapted to resist abrasion, which method includes forming a mold for the article, applying to grains of wear resisting material a coating of metal having a lower melting and alloying point than that of the metal forming the body of said article, distributing a layer of said previously coated grains on a surface of said mold adapted to shape 95 a surface of said article, and pouring molten metal into said mold.

9. The method of producing an article 100 adapted to resist abrasion, which method includes forming a mold for the article, applying a coating of tin to individual grains of wear resisting material, distributing a layer of said previously individually coated 105 grains on a surface of said mold adapted to shape a surface of said article, and pouring molten metal into said mold.

10. The method of producing an article 110 adapted to resist abrasion, which method includes forming a mold for the article, applying to grains of wear resisting material a coating of metal adapted to cling closely to the individual grains and having a lower alloying and melting point than that of the metal 115 forming the body of said article, distributing a layer of said previously coated grains on a surface of said mold adapted to shape a surface of said article, and pouring molten metal into said mold.

11. The method of producing an article 120 adapted to resist abrasion, which method includes forming a mold for the article, applying a thin coating of tin to grains of emery, distributing a layer of said previous- 125 ly coated grains on a surface of said mold adapted to shape a surface of said article, and pouring molten iron into said mold.

12. The method of producing an article 130 adapted to resist abrasion, which method

includes forming a mold for the article, applying mechanically a thin coating of tin to grains of emery, distributing a layer of said grains on a surface of said mold adapted to shape a surface of said article, and pouring molten iron into said mold.

13. The method of producing an article adapted to resist abrasion, which method includes forming a mold for the article, distributing on a surface of said mold adapted

to shape a surface of said article grains of wear-resisting material, said grains first having their surfaces roughened by fused alkali and then coated with metal, and pouring molten metal into said mold.

16 In testimony whereof, we have affixed our signatures hereto.

COLIN G. FINK.  
ARTHUR H. KOPP.